

# UNITED STATES PATENT OFFICE.

WILLIAM H. DAMON, OF LOS ANGELES, CALIFORNIA.

## NON-CUMULATIVE WAX POLISH.

1,240,544.

Specification of Letters Patent. Patented Sept. 18, 1917.

No Drawing. Application filed March 13, 1916, Serial No. 83,986. Renewed July 2, 1917. Serial No. 178,267.

*To all whom it may concern:*

Be it known that I, WILLIAM H. DAMON, a citizen of the United States of America, residing at Los Angeles, county of Los Angeles, State of California, have invented a certain new and useful Non-Cumulative Wax Polish; and I do hereby declare the following to be a full, clear, and exact description of the invention, such as will enable others skilled in the art to which it appertains to make and use the same.

This invention relates to a novel and improved non-cumulative wax polish which is more particularly adapted to be used to clean and polish varnished or enameled work or surfaces.

One object of the invention is to provide a novel and improved cleaning and polishing composition which contains no oil and which consists of an emulsion of water, soap, paraffin wax, turpentine, and rosin, combined with an abrasive; said composition being of such character that the wax is non-cumulative no matter how many different times the composition is applied to clean and polish the work or surface.

Further objects of the invention are to provide a novel and improved cleaning and polishing composition of the nature specified in which the ingredients remain permanently mixed and in suspension and form a homogenous mixture which can be used—without shaking—to clean, polish, and produce a coating or film of wax on, the work or surface; and leave the work or surface absolutely free from oil, and with a hard, glassy and perfect finish which is finger-mark proof, acid proof, dust proof, and weather proof, and can be washed by water without any bad effect on the finish.

Still further objects of the invention are to provide a novel and improved composition of the nature specified, which is highly effective for its purpose and adapted to produce quick and lasting results, with comparatively little rubbing, and which contains no ingredients at all harmful to even the finest varnish finished work or surface.

Other objects of the invention and the

advantages of the improved composition will be evident to those skilled in the art from a careful consideration of the description which follows.

The composition consists of the following ingredients: water, "Ivory" or other substantially pure soap, diatomaceous earth, spirits of turpentine, paraffin wax and rosin.

The proportions of the ingredients in the composition are approximately as follows:

|                       |              |    |
|-----------------------|--------------|----|
| Water                 | One gallon.  | 60 |
| Soap                  | Four ounces. |    |
| Diatomaceous earth    | Two pounds.  |    |
| Spirits of turpentine | One gallon.  |    |
| Paraffin wax          | Two pounds.  | 65 |
| Rosin                 | One ounce.   |    |

The water is first heated, then the soap is dissolved in the hot water, and then the diatomaceous earth is added and mixed with the soap and water. The paraffin wax and rosin are melted and added to the turpentine, and then the mixture of the wax, rosin, and turpentine are added to the mixture of the water, soap, and diatomaceous earth; and then all of the ingredients are thoroughly mixed together and agitated to form an emulsion.

The rosin rids the mixture of any free alkali and insures a higher degree of luster when the composition is applied in use. The wax hermetically seals and prevents checking and disintegration of the varnished work or surface.

The turpentine revivifies the varnish on the work or surface, and on each application of the composition to the work or surface the turpentine cuts the wax already on the work or surface so that the wax is non-cumulative on the work or surface, no matter how many times the composition is applied to clean and polish the work or surface. It will be understood that the composition may be applied to the work or surface by rubbing with cotton waste, cloth, chamois skin, etc.

I claim:

1. The herein-described cleaning and polishing composition consisting of water, soap,

diatomaceous earth, paraffin wax, spirits of turpentine, and rosin, substantially in the proportions specified.

2. A composition consisting of one gallon of water, four ounces of soap, two pounds of diatomaceous earth, one gallon of spirits of turpentine, two pounds of paraffin wax, and

one ounce of rosin, substantially as described and for the purposes specified.

In testimony whereof, I have signed my 10 name to this specification at Los Angeles, county of Los Angeles, State of California, this 6th day of March, A. D. 1916.

WILLIAM H. DAMON.